

## UNITED STATES PATENT OFFICE

GERALD U. GREENE, OF SALT LAKE CITY, UTAH, ASSIGNOR TO AMERICAN SMELTING AND REFINING COMPANY, OF NEW YORK, N. Y., A CORPORATION OF NEW JERSEY

## SEPARATION OF METALS

No Drawing.

Application filed August 8, 1929. Serial No. 384,474.

This invention relates to the separation of suitable apparatus, such as a bag-house. Any bismuth chlorides remaining in the metals, and more particularly to the removal of bismuth from ores, concentrates, compounds or various metallurgical products. Any bismuth chlorides remaining in the charge, together with substantially the entire content of copper chlorides, are soluble in certain acids and may be removed by 55 leaching the charge therein. The residue is thus freed from these elements and may be utilized as desired in the arts.

The invention also provides for the reduction of the copper content of the treated material to a sufficiently low value to render the material suitable for certain metallurgical purposes.

The invention provides for roasting the material containing bismuth and copper in the presence of a reagent which is capable of uniting with the bismuth and rendering the same volatilizable and of rendering the copper soluble in acid leaching solutions. The residue, after leaching, is low in bismuth and copper and may be used in various arts, such for example, as the manufacture of red lead or corroding lead.

The invention further consists in the new and novel features of operation and the new and original arrangements and combinations of steps in the process hereinafter described and more particularly set forth in the claims.

Although the novel features which are believed to be characteristic of this invention will be particularly pointed out in the claims appended hereto, the invention itself, as to its objects and advantages, the mode of its operation and the manner of its organization may be better understood by referring to the following description in which a particular commercial embodiment thereof is disclosed. It will be understood however, that the processes and the steps thereof may be modified 35 in various respects without departing from the broad spirit and scope of the invention.

In the following description and in the claims the various steps in the process and the details comprising the invention will be identified by specific names for convenience but they are intended to be as generic in their application as the art will permit.

The invention provides for the roasting of the bismuth and copper bearing materials in the presence of a chlorine compound and at a sufficiently high temperature to form chlorides of bismuth and copper. The bismuth chlorides are volatilized at the roasting temperature and may be recovered in any

mixing ores, concentrates, compounds or 60 other metallurgical products and particularly bismuth bearing materials with a small percentage of sodium chloride, after which they are roasted in any suitable furnace. The temperature of the roast or the chloridization 65 may be varied depending upon the percentage of lead. A temperature of some 450° to 600° C. has been found suitable for this purpose. The amount of sodium chloride required is also determined by the composition of the material and has been found to vary from 1% to 5%.

The bismuth, volatilized as bismuth chloride, is recovered in a suitable bag-house and the residue is leached, if desired, in dilute 75 sulphuric acid which removes the remainder of the bismuth and substantially the entire copper content.

As a specific example of the process a concentrate containing 2.52% bismuth, 38.1% 80 iron, 3.45% tin, 1.17% zinc and .3% lead was treated for one hour at a temperature of 600° C. with 2% of sodium chloride. It was found that 99.7% of the bismuth has been 85 volatilized.

As a further example, a lead concentrate containing 51.5% lead, and .18% bismuth was treated for one hour at a temperature of 420° C. with 3% sodium chloride. This resulted 90 in the volatilization of 77.6% of the bismuth.

A sample of smelter flue dust containing 53% lead and .45% bismuth was treated for thirty minutes with 5% sodium chloride at a temperature of 455° C. In this case 91.5% 95 of the bismuth was volatilized. It was found that the best results were secured when the temperature of chloridization ranged from 400° to 500° C. and the salt varied from 3% to 5% of the weight of the charge. Under

these conditions the bismuth was volatilized within one hour.

In carrying on the process as above, it was found that 98.1% of the copper is rendered soluble in sulphuric acid.

It is to be noted therefore that in processes requiring the complete elimination of copper the product may be used to advantage since the amount of copper which must be subsequently removed is reduced to a small value. After chloridization and leaching the bismuth has been reduced to .037% and the copper to slightly over 0.1%. The copper could of course be, recovered from the acid solution in any well known manner.

The lead is not volatilized to any appreciable extent during the salt roast provided the sulphur content of the charge is not excessive. If a large amount of sulphur in the sulphide form is present, the oxidization of the sulphur during the roasting operation may interfere with the temperature control and prevent proper regulation thereof. It is also to be noted that bismuth sulphate decomposes more readily than lead sulphate and at an appreciably lower temperature, whereas bismuth chloride has a slightly higher formation temperature than lead chloride. For this reason the bismuth chloride is formed in preference to lead chloride during the salt roast, thereby enabling the bismuth to be largely volatilized and removed without substantial loss of lead.

In the above described process the bismuth content of the material may be so treated that the product is suitable for corroding lead. For this purpose the bismuth is preferably reduced to .02%. In case it is desired to use the product for the manufacture of red lead, the elimination of the copper is a particularly important feature, as it would be necessary to remove this element by the use of additional reagents prior to manufacture of red lead. The process may be cheaply carried on, particularly in localities where salt may be easily obtained. It is to be understood that calcium chloride may be utilized instead of sodium chloride when that substance can be conveniently obtained.

Although certain novel features of the invention have been shown and described and are pointed out in the annexed claims, it will be understood that various omissions, substitutions and changes in the several steps of the process and in its operation may be made by those skilled in the art without departing from the spirit of the invention.

What is claimed is:

1. Process of treating lead bearing materials for the elimination of bismuth which comprises mixing said material with a small percentage of a chlorine compound and roasting the mixture at a temperature at which the bismuth is volatilized as a chloride without appreciable loss of lead.

2. Process of treating lead bearing materials for the elimination of bismuth which comprises mixing said material with a small percentage of sodium chloride and roasting the mixture at a temperature of 450° to 600° C. whereby the bismuth is volatilized as a chloride without appreciable loss of lead. 70

3. Process of treating lead bearing material for the elimination of bismuth which comprises mixing said material with from 1% to 5% of sodium chloride and roasting the mixture at a temperature of 450° to 600° C. whereby the bismuth is volatilized as a chloride without an appreciable loss of lead. 75

4. Process of treating lead bearing materials for the elimination of bismuth and copper which comprises chloridizing said materials at a temperature of 450° to 600° C. for a period of time sufficient to substantially completely volatilize the bismuth as a chloride, collecting and recovering said bismuth, leaching the material in a dilute acid solution whereby the copper and the remainder of the bismuth are largely removed and recovering the copper from the acid leach. 80

5. Process of treating lead bearing materials for the elimination of bismuth and copper which comprises chloridizing said materials at a temperature of 450° to 600° C. for a period of time sufficient to substantially 85 completely volatilize the bismuth as a chloride, collecting and recovering said bismuth, leaching the material in a sulphuric acid solution whereby the copper and the remainder of the bismuth are largely removed and recovering the copper from the acid leach. 90

6. Process of treating lead bearing materials for the elimination of bismuth which comprises chloridizing said materials at a temperature of 450° to 600° C. for a period 105 of time sufficient to substantially completely volatilize the bismuth as a chloride, collecting and recovering said bismuth, leaching the material in a dilute acid solution whereby the remainder of the bismuth is largely removed. 110

7. Process of treating lead bearing materials for the elimination of bismuth and copper which comprises chloridizing said materials at a temperature of 450° to 600° C. for a period of time sufficient to substantially 115 completely volatilize the bismuth as a chloride, and leaching the material in a dilute acid solution whereby the copper and the remainder of the bismuth are largely removed.

In testimony whereof I have hereunto set 120 my hand.

GERALD U. GREENE.